# EUROPEAN PATENT APPLICATION

(11) **EP 1 835 249 A1**
(43) Date of publication of application: **19.09.2007**
(21) Application number: 07002414.6
(22) Date of filing: 05.02.2007
(51) Int. Cl.: F26B 3/347, F26B 15/14, F26B 21/00

(54) **Drying apparatus, drying method of ceramic molded body and method for manufacturing honeycomb structured body**

(30) Priority: 17.03.2006 WO PCT/JP2006/305438
(71) Applicant: IBIDEN CO., LTD., Ogaki-shi Gifu 503-8604 (JP)
(72) Inventor: Kasai, Kenichiro Ibiden Co., Ltd., Ibi-gun Gifu 501-0695 (JP); Naruse, Kazuya, 45320 Courtenay (FR)
(74) Representative: HOFFMANN EITLE

(57) **Abstract**

It is an object of the present invention to provide a drying apparatus (10) capable of uniformly drying a ceramic molded body (1), and the drying apparatus of the present invention comprises:
a plurality of microwave irradiation parts (14a-14i) disposed alternately at the upper side and the lower side with respect to a conveying member (11) for conveying an item to be dried; and a plurality of hot air blowing parts (15a-15d), wherein the item to be dried is irradiated with microwaves in an alternating manner from the upper side and the lower side, hot air is applied in parallel with irradiation by the microwaves, to the item to be dried.

## Description

### TECHNICAL FIELD

The present invention relates to a drying apparatus, a drying method of a ceramic molded body, and a method for manufacturing a honeycomb structured body.

### BACKGROUND ART

Harm to the environment and the human body caused by particulates such as soot contained in exhaust gas discharged from the internal combustion engines of buses, trucks and other vehicles, construction equipment and the like has recently become a problem.
To remedy this, there are currently proposed numerous kinds of filters using a honeycomb structured body comprising porous ceramic as a filter for capturing particulates contained in exhaust gas, thereby purifying the exhaust gas.

Conventionally, when manufacturing a honeycomb structured body, for instance, first two kinds of ceramic powders having different average particle diameters, a binder, and a liquid dispersant are combined to prepare a wet mixture. This wet mixture is further mixed by using a screw mixing machine or the like, and then continuous extrusion molding is carried out using a die, and the extruded molded body is then cut to a prescribed length so that a rectangular pillar shaped honeycomb molded body is produced.

Next, the raw honeycomb molded body attained above is dried using microwave drying or hot-air drying, thereby manufacturing a dried body of a honeycomb molded body having a consistent degree of strength and which can be handled easily.

After the drying, prescribed cells are sealed to thereby achieve a plugged state of either end portion of the cells by a plug material layer. After the plugged state has been achieved, degreasing is carried out on the honeycomb molded body at a temperature in the range of 400 to 650 Degrees Celsius and under oxygen containing atmosphere to volatilize the solvent within the organic binder component while breaking down and eliminating resin components therein. Furthermore, firing is carried out on the honeycomb molded at a temperature in the range of 2000 to 2200 Degrees Celsius and under inert gas atmosphere thereby manufacturing the honeycomb fired body.

After this, a sealing material paste is applied to the side faces of the honeycomb fired bodies to adhere the honeycomb fired bodies together so that an aggregate of honeycomb fired bodies having a multitude of honeycomb fired bodies bonded together by interposing a sealing material layer (an adhesive layer) is manufactured. Then, cutting machine, or the like, to form a ceramic block of a prescribed form, such as cylindrical or cylindroid form and the like. Finally, sealing material paste is applied to the periphery of the ceramic block to form a sealing material layer (a coat layer), thus completing the manufacturing of the honeycomb structured body.

Also, when drying the honeycomb molded body in the method for manufacturing this kind of honeycomb structured body, there is known a drying method of a honeycomb molded body according to irradiating microwaves from a single direction (for example, see Patent Documents 1 and 2).

Patent Document 1: JP-A 2001-130970
Patent Document 2: JP-A 2005-131800

### DISCLOSURE OF THE INVENTION PROBLEMS TO BE SOLVED BY THE INVENTION

However, when drying the honeycomb molded body in the above mentioned manner, in a case of drying the honeycomb molded body according to irradiating microwaves from a single direction toward the honeycomb molded body, there has been the problem of it being easy for variation to occur in the moisture content of the dried honeycomb molded body according to the place therein, thereby making it easy for warpage to be generated caused by this kind of non-uniformity of dryness.
Further, there has also been a problem in which, in a case where the honeycomb fired body is manufactured by carrying out degreasing and firing on a honeycomb molded body in which uneven drying has progressed, the strength of the honeycomb fired body tends to be easily deteriorated.

### MEANS FOR SOLVING THE PROBLEMS

The inventors of the present invention have exacted keen examination in aim of solving the above mentioned problem, and have found that it is possible to achieve uniform drying of a ceramic molded body by carrying out drying by irradiating microwaves to the ceramic molded body in an alternating manner from the upper and lower sides, and further carrying out hot air drying in parallel with the microwave irradiation, and thus have perfected the drying apparatus, the drying method of a ceramic molded body and the method for manufacturing a honeycomb structured body of the present invention.

The drying apparatus of the present is a drying apparatus comprising: a plurality of microwave irradiation parts disposed alternately at the upper side and the lower side with respect to a conveying member for conveying an item to be dried; and a plurality of hot air blowing parts, wherein the item to be dried is irradiated with microwaves in an alternating manner from the upper side and the lower side, and hot air is applied in parallel with irradiation of the microwaves, to the item to be dried.

The drying method of a ceramic molded body of the present invention is a drying method of a ceramic molded body comprising passing a ceramic molded body through the interior of a drying apparatus to dry the ceramic molded body, the passing carried out in a prescribed period of time by using a conveying member, wherein the drying apparatus comprises: a plurality of microwave irradiation parts disposed alternately at the upper side and the lower side with respect to the conveying member; and a plurality of hot air blowing parts, and
the drying apparatus irradiates the ceramic molded body with microwaves in an alternating manner from the upper side and the lower side, and carries out a hot air drying in parallel with irradiation of the microwaves.

In the above mentioned drying method of a ceramic molded body of the present invention, it is preferable that the moisture content of the ceramic molded body after drying is 30% by weight or more and less than 70% by weight of the moisture content before drying.
It is also preferable in the above mentioned drying method of a ceramic molded body, that the temperature of the hot air is in a range of 40 to 80 Degrees Celsius.

The method for manufacturing a honeycomb structured body of the present invention is a method for manufacturing a honeycomb structured body comprising: manufacturing a pillar-shaped honeycomb molded body having a multiplicity of cells placed in parallel with one another in the longitudinal direction with a cell wall therebetween by molding a ceramic raw material; carrying out drying of a molded body comprising passing the honeycomb molded body through the interior of a drying apparatus to dry the honeycomb molded body, the passing carried out in a prescribed period of time with the honeycomb molded body placed onto a conveying member; and firing the dried honeycomb molded body to manufacture a honeycomb structured body comprising a honeycomb fired body, wherein the drying apparatus comprises: a plurality of microwave irradiation parts disposed alternately at the upper side and the lower side with respect to the conveying member; and a plurality of hot air blowing parts, and the drying apparatus irradiates the honeycomb molded body with microwaves in an alternating manner from the upper side and the lower side, and carries out a hot air drying in parallel with irradiation of the microwaves.

In the above mentioned method for manufacturing a honeycomb structured body of the present invention, it is preferable that the moisture content of the honeycomb molded body after drying is 30% by weight or more and less than 70% by weight of the moisture content before drying.
It is also preferable in the above mentioned method for manufacturing a honeycomb structured body, that the temperature of the hot air is in a range of 40 to 80 Degrees Celsius.

### EFFECTS OF THE INVENTION

According to the drying apparatus of the present invention, because it is possible to irradiate microwaves to the item to be dried in an alternating manner from the upper side and the lower side while applying hot air in parallel with the microwave irradiation, to the item to be dried, it is possible to achieve uniform drying of the items to be dried such as ceramic molded bodies. Therefore, in items to be dried which are dried using the drying apparatus of the present invention there is no occurrence of warpage or the like.

According to the drying method of a ceramic molded body of the present invention, because it is possible to irradiate microwaves to the ceramic molded body in an alternating manner from the upper side and the lower side while applying hot air in parallel with the microwave irradiation, to the ceramic molded body, it is possible to achieve uniform drying of the ceramic moldedbody, andbecauseof this, there is no occurrence of warpage or the like in the ceramic molded body after drying.

The method for manufacturing a honeycomb structured body of the present invention comprises drying to be carried out on the manufactured honeycomb molded body, and because in this process microwaves are irradiated to the honeycomb molded body in an alternating manner from the upper side and the lower side while applying hot air in parallel with the microwave irradiation, to the honeycomb molded body, it is possible to achieve uniform drying of the ceramic molded body, and because of this, there is no occurrence of warpage or the like in the honeycomb molded body after drying.
Because of this, it is possible to manufacture a honeycomb molded body of a prescribed shape with the method for manufacturing a honeycomb structured body of the present invention.
Also, because it is possible to achieve uniform drying of the honeycomb molded body with the method for manufacturing a honeycomb structured body of the present invention, it is possible to manufacture a honeycomb structured body comprising a honeycomb fired body having a high degree of strength.

### BEST MODE FOR CARRYING OUT THE INVENTION

Firstly, description will be given in regard to the drying apparatus and the drying method of a ceramic molded body according to the present invention.
The drying apparatus of the present is a drying apparatus comprising: a plurality of microwave irradiation parts disposed alternately at the upper side and the lower side with respect to a conveying member for conveying an item to be dried; and a plurality of hot air blowing parts, wherein the item to be dried is irradiated with microwaves in an alternating manner from the upper side and the lower side, and hot air is applied in parallel with irradiation of the microwaves, to the item to be dried.

The drying method of a ceramic molded body of the present invention is a drying method of a ceramic molded body comprising passing a ceramic molded body through the interior of a drying apparatus to dry the ceramic molded body, the passing carried out in a prescribed period of time by using a conveying member, wherein the drying apparatus comprises: a plurality of microwave irradiation parts disposed alternately at the upper side and the lower side with respect to the conveying member; and a plurality of hot air blowing parts, and
the drying apparatus irradiates the ceramic molded body with microwaves in an alternating manner from the upper side and the lower side, and carries out a hot air drying in parallel with irradiation of the microwaves.
Thus, it is possible for the drying method of a ceramic molded body of the present invention to optimally use the drying apparatus of the present invention.

Fig. 1 is a plan view showing a general representation of the drying apparatus of the present invention. Fig. 2(a) is a partial cross-sectional view taken along line A-A of the drying apparatus of the present invention shown in Fig. 1, and Fig. 2 (b) is a partial cross-sectional view taken along line B-B of the drying apparatus of the present invention shown in Fig. 1.
As shown in Fig. 1, a drying apparatus 10 comprises a drying furnace main body 19 including a conveying member for conveying an item to be dried (belt conveyor 11), microwave irradiation parts 14a to 14i disposed alternately at the upper side and the lower side with respect to the belt conveyor 11, a plurality of hot air blowing parts 15a to 15d established at a low position in a manner crawling along the floor and close to the belt conveyor 11, and hot air aspiration parts 15a' to 15d'; microwave transmission portions 13a to 13i joined to the microwave irradiation parts 14a to 14i by waveguide tubes 16a to 16i; and microwave leak prevention regions 12a and 12b disposed at the entrance side and exit side of the drying furnace main body 19 for the purpose of preventing the leakage of microwaves.
Therefore, with the drying apparatus 10 it is possible to carry out microwave irradiation on the item to be dried such as a ceramic molded body 1 from the upper side and the lower side alternately.

Moreover, as is shown in Figs. 2(a) and 2(b), the drying furnace main body 19 includes a microwave agitation blade 17 disposed on the ceiling portion of the drying furnace main body 19 for the purpose of uniformly irradiating microwaves from the microwave irradiation parts 14a to 14i to the item to be dried.
Therefore, according to rotating of the microwave agitation blade 17 it is possible to irradiate microwaves to the item to be dried in a uniform manner. Moreover, it is acceptable that the microwave agitation blade be provided in the drying apparatus of the present invention according to necessity.
Also, although the number of units or the location of installation of the microwave agitation blade 17 (not shown in Fig. 1) is not particularly limited, it is preferable that it be installed near the microwave irradiation parts (14b, 14c, 14f, 14h) used for the purpose of irradiating microwaves from the upper side with respect to the item to be dried.

In the drying apparatus 10, according to placing of the ceramic molded body 1 onto the belt conveyor 11, the ceramic molded body 1 is conveyed into the interior of the drying apparatus 10 through the entryway, and after a prescribed period of time has passed, is conveyed out through the exit of the drying apparatus 10.
Here, the belt conveyor 11 is set to move in an intermittent manner.

More specifically, the belt conveyor 11 is set in a manner so as to carry out a repeated operation of moving for at a prescribed speed for a prescribed period of time, then stopping momentarily for a prescribed period of time, and then moving again at a prescribed speed for a prescribed period of time. And for example, the belt conveyor 11 is set in such a manner that the hot air of the hot air blowing parts 15a to 15d inside of the drying apparatus 10 directly contacts the stationary ceramic molded body 1 in a direction parallel to the longitudinal direction of the ceramic molded body 1.
Moreover, in the drying apparatus of the present invention, it is not necessarily essential that the belt conveyor 11 (the conveying member for conveying an item to be dried) move intermittently, as it is also acceptable that the belt conveyor 11 be set to move continuously at a constant or varying speed.

Also, in the drying apparatus 10, the hot air aspiration parts 15a' to 15d' and the hot air blowing parts 15a to 15d are disposed in an opposing manner, and because of this, it is possible to blow the hot air to the longitudinal direction of the ceramic molded body in a more precise manner.
It is not however absolutely essential that the above mentioned hot air aspiration parts be provided.

The drying method of a ceramic molded body of the present invention can be carried out using this kind of drying apparatus of the present invention.
Here, description will be given in regard to desirable drying conditions and the like using as an example a case of using a pillar-shaped honeycomb molded having a multiplicity of cells placed in parallel with one another in the longitudinal direction with a cell wall therebetween as the ceramic molded body serving as the item to be dried.
It is a matter of course that the item to be dried in the drying method of the present invention is not limited to being a honeycomb molded body, as various kinds of ceramic molded bodies may also serve as items to be dried.
In the present specification, the shape indicated by the word "pillar" refers to any desired shape of a pillar including a round pillar, an oval pillar, a polygonal pillar and the like.

In the drying method of the present invention, microwaves are irradiated alternately from the upper side and the lower side with respect to the honeycomb molded body while hot air drying is conducted in parallel with irradiation of microwaves.
In this manner, according to irradiating microwaves alternately from the upper side and the lower side with respect to the honeycomb molded body, because the moisture located throughout the honeycomb molded body is eliminated uniformly, there is no occurrence of warpage or the like in the honeycomb moldedbodyafterdrying. Also, because hot air drying is carried out in parallel with the microwave irradiation, it is possible to avoid the inconvenience of warpage had in cases of drying according to only microwave irradiation, as cases of drying according to only microwave irradiation have a trend of it being difficult to achieve a dried state at areas near the central portion of the honeycomb molded body, and as a result there is a concern that there will be slight generation of warpage in the honeycomb molded body. Moreover, in light of the above, it is preferable that the ceramic molded body dried with the drying method of the present invention be the above mentioned honeycomb molded body.

Also, the drying apparatus 10 shown in Fig. 1 includes four microwave irradiation parts (14b, 14c, 14f, 14h) for the purpose of irradiating microwaves from the upper side with respect to the honeycomb molded body, and five microwave irradiation parts (14a, 14d, 14e, 14g, 14i) for the purpose of irradiating microwaves from the lower side with respect to the honeycomb molded body. The number of microwave irradiation parts for the purpose of irradiating microwaves from the lower side with respect to the honeycomb molded body is greater than the number of microwave irradiation parts for the purpose of irradiating microwaves from the upper side with respect to the honeycomb molded body. The reason for this is that in a case in which microwaves are irradiated to the honeycomb molded body from the lower side, microwaves must pass through the belt conveyor to irradiate the honeycomb molded body, which tends to lead to difficulty in drying the bottom of the honeycomb molded body.
It is however acceptable for the number of the microwave irradiation parts at the upper side and the lower side to be the same, and it is also acceptable for the number of the microwave irradiation parts disposed at the upper side to be greater than that of the lower side.
It is also acceptable to have the number of the microwave irradiation parts at the upper side and the lower side to be the same while having the microwaves irradiated from the lower side with respect to the honeycomb molded body set to a higher power.
Although the specific number of the abovementionedmicrowave irradiation parts is not particularly limited, it is preferable that there be two or more microwave irradiation parts disposed at the upper side with respect to the item to be dried and three or more microwave irradiation parts disposed at the lower side with respect to the item to be dried.

Also, while it is not possible to indiscriminately regulate the conditions of power and the like of the microwaves in the drying method of the present invention due to the conditions and the like being dependant upon factors such as the shape and size of the ceramic molded body or the like, which is the subject of drying (the item to be dried), it is for example desirable for the power of the microwave irradiated from each microwave irradiation part to be in the range of 3 to 7 kW, and even more desirable at 5kW, in a case of drying a honeycomb molded body (ceramic molded body) which is to become a honeycomb fired body having a dimension of 33 mm × 33 mm × 300 mm, the number of cells of 31 pcs/cm², and cell wall thickness of 0.35mm after firing.

Also, as has already been described, although it is acceptable for the honeycomb molded body to be moved by the belt conveyor either intermittently or continuously, it is desirable that it be moved intermittently.
And in such a case, it is preferable that the movement speed of the belt conveyor is 2 to 8 m/min. Also, it is preferable that the period of time over which the belt conveyor is stopped be at almost two seconds. Moreover, the movement speed of the above mentioned belt conveyor is not differentiated according to moving time and stopping time, but is calculated as the amount of movement per unit of time.

Also, it is preferable that the period of time (drying time) over which the honeycomb molded body exists inside of the drying apparatus be in the range of 2 to 3 minutes. If the drying time is less than two minutes, there are cases in which drying is insufficient, and on the other hand if the drying time exceeds three minutes, there are cases in which drying progresses excessively causing warpage and the like to occur.

Also, in the drying method of the present invention, it is preferable that the moisture content of the ceramic molded body (honeycomb molded body) after drying is 30% by weight or more and less than 70% by weight of the moisture content before drying. If the moisture content after drying is less than 30% by weight of the moisture content before drying, the moisture content within the honeycomb molded body is insufficient, which may lead to the occurrence of warpage, cracks, or the like in the honeycomb moldedbody. And furthermore, if the moisture content is reduced to less than 30% by weight, the microwaves come to be absorbed into the ceramic powder leading to a sudden rise in the temperature of the ceramic powder within the honeycomb molded body which thereby starts degreasing. Alternately, if the moisture content after drying is 70% weight or more of the moisture content before drying, drying is insufficient, which leads to a deterioration of the degree of handleability normally enjoyed.
It is possible to adjust the moisture content after drying by adjusting the of drying time, the power of the microwaves, the temperature of the hot air, and the like.

Also, in the above mentioned drying method, it is preferable that the temperature of the hot air is in the range of 40 to 80 Degrees Celsius. This is because at a temperature of less than 40 Degrees Celsius, there are cases in which it is impossible to enjoy the effects attained by the additional use of the hot air that has been described herein above. And alternately, at a temperature exceeding 80 Degrees Celsius there are cases in which state of drying progresses sharply causing the occurrence of warpage, cracks, and the like in the ceramic molded body (honeycomb molded body).

Moreover, it is preferable that the airspeed of the above mentioned hot air is in the range of 20 to 40 m/sec.
If the above mentioned airspeed is less than 20 m/sec the drying speed tends to become slow, giving rise to occurrences of drying variation in the ceramic molded body. And if the above mentioned airspeed exceeds 40 m/sec there are cases in which drying progresses excessively at only the surface of the ceramic molded body.
By using this kind of drying method, it is possible to dry the ceramic molded body in a manner setting the moisture content thereof to a desired amount and without occurrences of warpage or cracks.

Next, description will be given in regard to the method for manufacturing a honeycomb structured body of the present invention.
The method for manufacturing a honeycomb structured body of the present invention is a method for manufacturing a honeycomb structured body comprising: manufacturing a pillar-shaped honeycomb molded body having a multiplicity of cells placed in parallel with one another in the longitudinal direction with a cell wall therebetween by molding a ceramic raw material; carrying out drying of a molded body comprising passing the honeycomb molded body through the interior of a drying apparatus to dry the honeycomb molded body, the passing carried out in a prescribed period of time with the honeycomb molded body placed onto a conveying member; and firing the dried honeycomb molded body to manufacture a honeycomb structured body comprising a honeycomb fired body, wherein the drying apparatus comprises: a plurality of microwave irradiation parts disposed alternately at the upper side and the lower side with respect to the conveying member; and a plurality of hot air blowing parts, and the drying apparatus irradiates the honeycomb molded body with microwaves in an alternating manner from the upper side and the lower side, and carries out a hot air drying in parallel with irradiation of the microwaves.

Fig. 4 is a perspective view schematically showing an example of a honeycomb structured body. Fig. 5(a) is a perspective view schematically showing a honeycomb fired body which comprises the above mentioned honeycomb structured body, while Fig. 5 (b) is a cross-sectional view taken along line A-A thereof.

Normally, in a honeycomb structured body 130, a plurality of honeycomb fired bodies 140 of the kind shown in Figs. 5 (a) and 5 (b), are bound together by interposing a sealing material layer (an adhesive layer) 131 forming a ceramic block 133, and a sealing material layer (a coat layer) 132 is further formed on the periphery of the ceramic block 133. In the honeycomb fired body 140, as shown in Fig. 4, a multitude of cells 141 are placed in parallel with one another in the longitudinal direction, and a cell wall 143, which separates the cells 141 from one another is allowed to function as a filter.

More specifically, as shown in Fig. 5(b), the end portion of either the exhaust gas inlet side or the exhaust gas outlet side of the cells 141 formed in the honeycomb fired body 140 is sealed by a plug material layer 142. Therefore, exhaust gas entering one cell 141 will always pass through the cell wall 143 separating the cells 141 and thus flow out through another one of the cells 141. When the exhaust gas passes through the cell wall 143, particulates contained within the exhaust gas are captured by the cell wall 143, thereby purifying the exhaust gas.
Because this kind of honeycomb structured body 130 comprises honeycomb fired bodies 140 that are made of silicon carbide and thus excel extremely in thermal resistance and are easily regenerated, it is used in various types of large scales vehicles and diesel engine equipped vehicles and the like.

Hereinbelow, description will be set forth in regard to the method for manufacturing a honeycomb structured body of the present invention, in process order.
At this point, using as an example a case of manufacturing a honeycomb structured body having silicon carbide as a main component, description will be put forth in regard to the method for manufacturing a honeycomb structured body of the present invention.
It is a matter of course that the main component of the constituting material of the honeycomb structured body is not limited to silicon carbide. Other examples of the material include for instance, components such as nitride ceramics such as aluminum nitride, silicon nitride, boron nitride, titanium nitride; carbide ceramics such as zirconium carbide, titanium carbide, tantalum carbide, tungsten carbide; and oxide ceramics such as alumina, zirconia, cordierite, mullite, and aluminum titanate, and the like.
Out of the above mentioned possible components, non-oxide ceramics are desirably used, with silicon carbide being particularly desirable. This is because they are excellent in thermal resistance properties, mechanical strength, and thermal conductivity. Moreover, silicon-containing ceramic, which is had by infusing metallic silicon with the ceramics set forth above, as well as ceramic bound by silicon or silicate compounds can also be used as the constituting material of the honeycomb structured body. And out of these, those (silicon-containing silicon carbide) of silicon carbide with metallic silicon are preferable.

First, organic binder is dry mixed with an inorganic powder such as silicon carbide powder having a varying average particle' diameter as a mixed powder. While the mixed powder is being prepared, a mixed solution is prepared of blended liquid plasticizer, lubricant, and water. Next, the above mentioned mixed powder and the above mentioned mixed solution are further blended together using a wet mixing machine, and thus a wet mixture for use in manufacturing the molded body is prepared.

Now although the particle diameter of the above mentioned silicon carbide powder is not particularly limited, a particle diameter having little shrinkage during the subsequent firing is preferable. For example, a powder mix of 100 parts by weight of a powder having an average particle diameter in the range of 0.3 to 50 µm, and 5 to 65 parts by weight of another powder having an average particle diameter in the range of 0.1 to 1.0 µm, is desirable.
Although in order to adjust the pore diameter of the honeycomb molded body, it is necessary to adjust the firing temperature, the pore diameter can also be adjusted by adjusting the particle diameter of the inorganic powder.

The above mentioned organic binder is not limited in particular, and binders such as methylcellulose, carboxymethyl cellulose, hydroxyethyl cellulose, polyethylene glycol, for example, are acceptable for use therein. Of the binders mentioned above, methylcellulose is the most preferable.
It is preferable that the above mentioned binder be blended with the inorganic powder at a ratio of 1 to 10 parts by weight per 100 parts by weight of inorganic powder.

The above mentioned plasticizer is not limited in particular, and substances such as glycerin, for example, are acceptable for use as such.
The above mentioned lubricant is not limited in particular, and substances such as polyoxyalkylene-based compounds such as polyoxyethelyne alkyl ether, and polyoxypropylene alkyl ether, for example, are acceptable for use as such.
Some concrete examples of lubricants are substances such as polyoxyethelyn monobutyl ether, and polyoxypropylene monobutyl ether.
Also, in some cases, it is unnecessary to use plasticizer or lubricant in the mixed material powder.

Also, when preparing the above mentioned wet mixture, it is acceptable to use a dispersant such as water, organic solvents such as benzol, and alcohol such as methanol and the like, for example.
Further, it is also acceptable to add a mold aiding agent to the above mentioned wet mixture.
The mold aiding agent is not limited in particular, and substances such as ethylene glycol, dextrin, fatty acids, fatty acid soap, or poly alcohol, for example, may be used.

Further, it is acceptable, according to need, to add a pore-forming agent such as balloon, which is a micro sized hollow sphere having oxide-based ceramic as a component therein, in addition to spherical acrylic particle, or graphite, to the above mentioned wet mixture.
The above mentioned balloon is not particularly limited, and alumina balloons, glass micro balloons, shirasu balloons, fly ash balloons (FA balloons), mullite balloons and the like, for example, are all acceptable for use. Of the above mentioned, alumina balloon is the most preferable for use.

Also, it is preferable for the temperature of the above prepared wet mixture, which uses silicon carbide powder, to be 28 Degrees Celsius or less. This is because if the temperature is too high, organic binder will undergo gelatinization.
It is also preferable for the inorganic ratio of within the above mentioned wet mixture to be 10% by weight or less, and it is also preferable for the moisture content weight of the same wet mixture to be in the range of 8.0 to 20.0% by weight.

After preparation, the above mentioned wet mixture is inducted into an extrusion-molding machine, and according to extrusion-molding, a pillar-shaped honeycomb molded having a multiplicity of cells placed in parallel with one another in the longitudinal direction with a cell wall therebetween is produced.
Afterward, drying of a molded body is carried out on this honeycomb molded body by placing it onto a conveying member which thereby passes the honeycomb molded body through the interior of the drying apparatus in a prescribed period of time, so that the honeycomb molded body is dried.
Here, the honeycomb molded body is dried according to the drying method of the present invention which uses the drying apparatus of the present invention. And since the drying method has already been described in detail herein above, that same detailed description will be omitted at this point.
And, because the above mentioned drying method is employed into use in the present process in the method for manufacturing a honeycomb structured body of the present invention, it is possible to dry the honeycomb molded body uniformly and without occurrences of warpage and the like regardless of the composition (the kind of ceramic, the kind of binder or the like) of the wet mixture constituting the honeycomb molded body.

Also, in the above mentioned drying of a molded body, it is preferable that the moisture content of the honeycomb molded body after drying is 30% by weight or more and less than 70% by weight of the moisture content before drying.
In the present process, according to drying the honeycomb molded body, the degree of handleability of the honeycomb molded body was difficult due to the honeycomb molded body being easily prone to deformation due to the moisture content of the honeycomb molded body of directly after molding being high. In contrast to this, in the present process, according to drying the honeycomb molded body, thereby reducing the moisture content in the molded body, the degree of handleability is improved. Because of this, in the present process, it is preferable that the moisture content of the honeycomb molded body after drying be set to less than 70% by weight of the moisture content before drying.
Also, the reason that it is preferable to set the moisture content of the above mentioned honeycomb molded body after drying to 30% by weight or more is that if the moisture amount is reduced to below this amount there arises the concern of the occurrence of warpage, cracks, or the like in the honeycomb molded body, and furthermore, the microwaves come to be absorbed into the ceramic powder leading to a sudden rise in the temperature of the ceramic powder within the honeycomb molded body which thereby starts degreasing.

It is also preferable in the above mentioned drying of a molded body, that the temperature of the hot air is in a range of 40 to 80 Degrees Celsius. The reason for this is as was set forth herein above.

Next, it is preferable to carry out further drying in order to nearly completely eliminate the moisture within the above mentioned honeycomb molded body, and here, in the state of the honeycomb molded body being held by a drying jig, it is preferable to carry out drying using a hot air drying apparatus.

Fig. 3 is a cross-sectional view schematically showing an example of the above mentioned drying jig.
As shown in Fig. 3, a drying jig 20 comprises two jigs, a top jig 21 and a bottom jig 22. The top jig 21 is fabricated in a manner joining the long sides of two long and thin plate shaped bodies in a manner such that their main faces are orthogonal, and the bottom jig 22 has a shape identical to the top jig 21.
Disposed to the top jig 21, as shown in Fig. 3, is a fixing member 23 for the purpose of fixing the top jig 21 and the bottom jig 22 after they have been combined. It is acceptable to dispose the fixing member onto the top jig, as it is also acceptable to dispose the fixing member onto the bottom jig.

This fixing member 23 comprises a fixing piece 23a fixed onto the plate shaped body using a screw, and a holding piece 23b installed via a spring 23c onto the fixation piece 23a in a rotatable manner. As is shown in Fig. 3, the fixing member 23 can exist in a fixed state in which the holding piece 23b holds down the bottom jig 22 thus fixing it in place, as well as a released state in which the holding piece 23b is collapsed in a direction roughly identical to the fixing piece 23a. In the fixation member 23, if the top end of the holding piece 23b in the released state is moved a certain distance toward the outside (in the direction running away from the fixing piece 23a) the holding piece 23b switches to the fixed state to firmly hold down and fix the bottom jig 22 in place. Alternately, if the holding piece 23b in the fixed state is moved a certain distance toward the inside (in the direction nearing the fixation piece 23a), the holding piece 23b switches to the released state.

As has been set forth herein above, in the drying used for the purpose of nearly completely eliminating the moisture within the honeycomb molded body, it is preferable to conduct a drying treatment in which the honeycomb molded body 1 is held by a drying jig 20 of the kind shown in Fig. 3.
By using this kind of drying jig in a state of the drying jig compressing the honeycomb molded body from the sides while fixing it in place so that the shape does not change, it is possible to carry out drying on the honeycomb molded body in such a state that there is almost no moisture therein as well as no occurrence of warpage and the like.

And although the drying jig 20 shown in Fig. 3 comprises two separatable jig members, the drying jig used in the present invention can also be comprised of a single openable and closable jig member.
And it is also acceptable that the above mentioned drying jig be able to be used in a manner stacked in multiple levels such as two levels, as it is also acceptable for it to be used as a single level only.

Next, cells are sealedaccordingtoneed. Here, a prescribed amount of plug material paste, which becomes the actual plug, is filled into the end portions of the outlet sides of the inlet side cell group, as well as the end portions of the inlet sides of the outlet side cell group.
Although the above mentioned plug material paste is not particularly limited, it is preferable that the plug manufactured through the subsequent processes exhibits a porosity in the range of 30 to 70%. It is for instance, possible to use a material that is the same as the above mentioned wet mixture as the plug material paste.

It is acceptable to carry out filling of the above mentioned plug material paste according to necessity, and in a case of carrying out filling of the above mentioned plug material paste, it is possible to use the honeycomb structured body attained through the subsequent processes optimally as a honeycomb filter, for instance. And in a case of not having had filled the above mentioned plug material paste into the cells, it is possible to use the honeycomb structured body attained through the subsequent processes optimally as a catalyst supporting carrier, for instance.

Next, by carrying out degreasing (at 200 to 500 Degrees Celsius, for example) and firing (at 1400 to 2300 Degrees Celsius, for example) under prescribed conditions on a honeycomb molded body in which with the above mentioned plug material paste is filled, it is possible to manufacture a pillar shaped honeycomb fired body in which one of the end portions of the above mentioned cells are plugged, and a multitude of cells are placed in parallel with one another in the longitudinal direction with a cell wall therebetween.
The above mentioned conditions under which degreasing and firing are executed to the above mentioned honeycomb molded body can be the same conditions that have been used conventionally when manufacturing a filter comprised of porous ceramic.

Next, a sealing material paste, which becomes the sealing material layer (the adhesive layer) is applied to the side surfaces of the honeycomb fired body in a uniform thickness. After this, another honeycomb fired body is successively stacked to the sealing material paste layer. By carrying out the above process repeatedly, an aggregate of honeycomb firedbodies having a prescribed size is produced.

It is possible to use a substance such as a substance containing inorganic fiber and/or inorganic particle in addition to inorganic binder, organic binder, for example, as the above mentioned sealing material paste.
It is acceptable to use silica sol, alumina sol, and the like, for example, as the above mentioned inorganic binder. Also, it is acceptable to use the above singly, or use a combination of two or more of them in parallel. Of the above mentioned inorganic binders, silica sol is most preferable for use.

It is acceptable to use polyvinyl alcohol, methylcellulose, ethylcellulose, carboxy methylcellulose, and the like, for example, as the above mentioned organic binder. Also, it is acceptable to use the above singly, or use a combination of two or more of them in parallel. Of the above mentioned organic binders, carboxy methylcellulose is most preferable for use.

It is acceptable to use ceramic fibers such as silica-alumina, mullite, alumina, silica, for example, as the above mentioned inorganic fiber. Also, it is acceptable to use the above singly, or use a combination of two or more of them in parallel. Of the above mentioned inorganic fiber, alumina fiber is most preferable for use.

It is acceptable to use carbide, nitride, and the like, for example, as the above mentioned inorganic particle. More specifically, it is acceptable to use inorganic powder and the like comprising silicon carbide,silicon nitride,boron nitride, or the like, for example, as the above mentioned inorganic particle. It is acceptable to use the above singly, or use a combination of two or more of them in parallel. Of the above mentioned inorganic particle, silicon carbide, which excels in its thermal conductivity properties, is most preferable for use.

And furthermore, it is also acceptable, according to need, to add a pore-forming agent such as balloon which is a micro sized hollow sphere having oxide based ceramic as a component therein, and spherical acrylic particle, or graphite and the like, to the above mentioned sealing material paste.
The above mentioned balloon is not particularly limited, and alumina balloon, glass micro balloon, shirasu balloon, fly ash balloon (FA balloon), mullite balloon, and the like, for example, are all acceptable for use. Of the above mentioned, alumina balloon is the most preferable for use.

Next, this aggregate of honeycomb fired bodies is heated to dry the sealing material paste layer, which then hardens to become the sealing material layer (the adhesive layer).
Next, using a diamond cutter or the like, cutting is carried out on the aggregate of honeycomb fired bodies, which comprises a plurality of honeycomb fired bodies adhered together by interposing the sealing material layer (the adhesive layer), thereby producing a cylindrical ceramic block.

Afterward, another sealing material layer (a coat layer) is formed by coating the above mentioned sealing material paste to the outer periphery of the ceramic block. Thus, a honeycomb structured body having the sealing material layer (the coat layer) formed on the outer peripheral portion of a cylindrical ceramic block comprising a plurality of honeycomb fired bodies adhered together by interposing the sealing material layer (the adhesive layer) is manufactured.

Afterward, a catalyst is supported on the honeycomb structured body as needed. It is also acceptable to support the above mentioned catalyst onto the honeycomb fired bodies, before the honeycomb fired bodies are manufactured into the honeycomb molded body aggregate.
In a case where the catalyst is supported, it is preferable that a film of alumina, which has a high specific surface area, be formed onto the surface of the honeycomb structured body, and a co-catalyst and a catalyst such as platinum and the like is adhered to the surface of the alumina film.

It is acceptable to apply a method of impregnating the honeycomb structured body with a metallic compound containing an aluminum species such as Al (NO₃) and the like, for example, and then heating, or a method of impregnating the honeycomb structured body with a solution containing alumina powder and then heating and other methods, as a method of forming the alumina film onto the surface of the above mentioned honeycomb structured body.
It is acceptable to apply a method of impregnating the honeycomb structured body with a metallic compound containing a rare earth element such as Ce (NO₃) ₃ and the like, for example, and then heating, as a method of administering the co-catalyst onto the above mentioned alumina film.
It is acceptable to apply a method of impregnating the honeycomb structured body with a substance such as a dinitrodiammine platinum nitric acid solution ([Pt (NH₃) ₂ (NO₂) ₂ HNO₃, platinum content 4.53% by weight) and the like, for example, and then heating and other methods, as a method of adhering the catalyst onto the above mentioned alumina film.
Also, it is acceptable that the catalyst is adhered with a method of first adhering the catalyst to alumina particles in advance, and subsequently impregnating the honeycomb structured body with the solution containing the alumina powder, to which the catalyst has been adhered in advance.

In the method for manufacturing a honeycomb structured body put forth up to this point, although the honeycomb structured body has been a honeycomb structured body (also termed "aggregated honeycomb structured body" hereinafter) having a form of a plurality of honeycomb fired bodies bound together by interposing the sealing material layer (the adhesive layer), the honeycomb structured body manufactured according to the method for manufacturing a honeycomb structured body of the present invention can also be a honeycomb structured body (also termed "integral honeycomb structured body" hereinafter) having a form of a honeycomb firedbody configured as a single cylindrical ceramic block.

In a case of manufacturing an integral honeycomb structured body of this sort, the only aspect that is different than a case of manufacturing the aggregated honeycomb structured body is that the size of the honeycomb molded body, that is extrusion molded, is larger in the case of manufacturing an integral honeycomb structured body than that in the case of manufacturing an aggregated honeycomb structured body, and all other aspects used to manufacture an integral honeycomb structured body are identical to those used in manufacturing an aggregated honeycomb structured body.
At this point, because the methods and the like by which the wet mixture of before molding is conveyed and stored are identical to those in the method of manufacturing the 6 mentioned aggregated honeycomb structured body, description thereof will be omitted.

Next, in the same manner as in the method of manufacturing an aggregated honeycomb structured body, the above mentioned honeycomb molded body is dried out using the drying method of the present invention employing the drying apparatus of the present invention. Moreover, according to need, it is acceptable to carry out the drying for the purpose of nearly completely eliminating the moisture from the honeycomb molded body. Next, cells are sealed by filling a prescribed amount of plug material paste into the end portions of the outlet sides of the inlet side cell group, as well as the end portions of the inlet sides of the outlet side cell group.
Afterward, in the same manner as in the manufacture of the aggregated honeycomb structured body, degreasing and firing are carried out, thereby producing a ceramic block. And according to need, it is possible to form the sealing material layer (the coat layer). Thus, an integral honeycomb structured body is manufactured. Further, it is also acceptable to support a catalyst on the above mentioned integral honeycomb structured body with the method put forth herein above.

In the case of manufacturing the honeycomb structured body according to the manufacturing method set forth herein above, when manufacturing the above mentioned aggregated honeycomb structured body, it is desirable to use silicon carbide or silicon-containing silicon carbide powder as the main component of the constituting material, and when manufacturing the integral honeycomb structured body it is desirable to use cordierite or aluminum titanate as the main component of the constituting material.

Also, although description has been centered mainly around the honeycomb filter, for the purpose of capturing particulates in the exhaust gas, as the honeycomb structured body, the above mentioned honeycomb structured body can also be used suitably as a catalyst supporting carrier (honeycomb catalyst) for converting exhaust gas.
With the herein above described method for manufacturing a honeycomb structured body of the present invention it is possible to optimally manufacture a honeycomb structured body having a prescribed shape.

### EXAMPLES

Herein below examples will be set forth describing the present invention in further detail, though it should be understood that the present invention is not limited to these examples.

### (Example 1)

(1) First, 250kg of α-type silicon carbide powder having an average particle diameter of 10 µm, 100kg of α-type silicon carbide powder having an average particle diameter of 0.5 µm, and 20kg of organic binder (methylcellulose) were blended together to prepare a powder mixture.
Next, 12kg of lubricant (UNILUB, manufactured by NOF Corp.), 5kg of plasticizer (glycerin), and 65kg of water were blended in a separate container to prepare a liquidmixture. Next, using a wet mixing machine, the powder mixture and the liquid mixture were blended together, thereby preparing the wet mixture.
Next, extrusion-molding using this wet mixture, and cutting following the extrusion-molding was carried out, and thereby a honeycomb molded body was produced.

(2) Next, the above mentioned honeycomb molded body was dried using the drying apparatus 10 shown in Figs. 1 and 2, wherein the moisture content (remaining moisture ratio) of the honeycomb molded body was set to 50% by weight of the moisture content before drying.
Morespecifically,theabovementioned honeycomb molded body was dried by running a repeated operation of moving the belt conveyor 11 for two seconds at a speed of 4.5 m/min through the interior of the drying furnace main body 19 which has a movement distance of 15 m, and then stopping the belt conveyor 11 for two seconds, whereby the honeycomb molded body was conveyed intermittently, duringwhich, the honeycomb molded body was dried by irradiating 5.0 kW microwaves from each of the microwave irradiation parts disposed at the upper side and the lower side with respect to the drying furnace interior while blowing 50 Degrees Celsius hot air at an airspeed of 30 m/sec from each of the hot air blowing parts.
Also, the remaining moisture ratio of the honeycomb molded body was calculated based on the mass change of the moisture content of before and after drying.

(3) Next, a drying treatment in the manner below was carried out.
The honeycomb molded body was held by the drying jig (made of epoxy resin) shown in Fig. 3, and drying was carried out by carrying in this drying jig in a state of it being stacked as two levels into a hot air drying apparatus.
The drying conditions here were as follows: the temperature of the interior of the drying apparatus was set to a 100 Degrees Celsius, and the time spent inside of the drying apparatus was set to 15 minutes.

(4) Next, the honeycomb molded body on which the above mentioned drying treatment had been carried out was removed from the drying jig, and a plug material paste having a constitution identical to the above mentioned wet mixture was filled into prescribed cells.
Next, after carrying out further drying by using a drying apparatus, degreasing was carried out at 400 Degrees Celsius, and firing was carried out for three hours at atmospheric pressure in an argon atmosphere at 2200 Degrees Celsius, thereby manufacturing a honeycomb sintered body made from a silicon carbide sintered body having a porosity of 40%, an average pore diameter of 12.5 µm, dimensions of 34.3 mm × 34.3 mm × 305 mm, the number of cells (cell density) of 46.5 pcs/cm², and a cell wall thickness of 0.25 mm.

### (Examples 2 to 10, Reference Examples 1 to 5)

In the process (2) of Example 1, aside from the point of having changed the drying conditions to those indicated in Table 1, and having produced the honeycomb molded body exhibiting a moisture after drying with respect to the moisture content before drying of the value indicated in Table 1, the honeycomb fired body was manufactured in a manner identical to the Example 1.

### (Comparative Example 1)

In the process (2) of Example 1, when drying the honeycomb molded body using the drying apparatus 10, aside from the point of irradiating microwaves from only the microwave irradiation parts (14b, 14c, 14f, 14h) disposed at the upper side with respect to the conveyor member (the belt conveyor 11) to dry the honeycomb molded body with the conditions indicated in Table 1, the honeycomb fired body was manufactured in a manner identical to the Example 1.
In this Comparative Example, it can be said that irradiation of the microwaves is carried out only from the upper side with respect to the honeycomb molded body.

For each Example, Reference Example, and Comparative Example, after the honeycomb molded body is dried, the handleability of the molded body after drying was evaluated with the method set forth below, and furthermore, the amount of warpage of the produced honeycomb fired body was measured. The results are shown in Table 1.

### (Evaluation of handleability)

An evaluation of the handleability of the honeycomb molded body was conducted using a handleability evaluation jig (see Figs. 6(a) and 6(b)).
As an evaluation tool, a handleability evaluation jig 50 was used. The handleability evaluation jig 50 is constituted by two flat plate shaped bodies 51 that are slightly larger than the side faces of the honeycomb molded body 1, each plate shaped body having a urethane layer 51a formed on the entirety of one of the main faces, wherein the two urethane layers 51a face each other.
And in the evaluation, first, the honeycomb molded body 1 was placed between the two plate shaped bodies 51, after which each one of the above mentioned plate shaped bodies 51 is pressed to the corresponding parallel side face of the honeycomb molded body 1 at a pressure of 2 kPa to thereby sandwich the honeycomb molded body 1. Afterward, the amount of deformation of the honeycomb molded body 1 was measured and handleability was thereby evaluated with the following evaluation standard.

That is, in a state sandwiching the honeycomb molded body 1 with the two plate shaped bodies 51 as shown in Fig. 6(b), with respect to the end face of the honeycomb molded body 1, the length (the length of the portion sandwiched by the arrows in Fig. 6 (b)) of a portion therein which has an equal distance from the main faces of each of the two plate shaped bodies was measured, and the measured length was compared with the length of the same portion of the honeycomb molded body before being sandwiched by the two plate shaped bodies 51 and the difference in the length was referred to as the amount of deformation.
As the evaluation standard, "o" represents absolutely no deformation, "Δ" represents an amount of deformation of less than 1mm, and "x" represents an amount of deformation of 1mm or more.

### (Measurement of the amount of warpage)

Measurement of the amount of warpage of the honeycomb fired body was carried out using a warpage amount measurement jig.
The warpage amount measurement jig is constituted by a straight block member having a length roughly identical to the full length of the honeycomb fired body, and contact members of the same thickness established on both ends of the block member , and has installed on the center of this block member a scale (a scale for warpage measurement) slidable in the direction perpendicular to the longitudinal direction of the above mentioned block member.
And during measurement, the above mentioned contact members are made to contact near both ends of the dried honeycomb fired body, and afterward, the scale for warpage measurement is moved to the fired body, where the amount of movement of the scale at the time the above mentioned scale makes contact with the fired body is read. According to doing this, the amount of warpage was carried out.

**Table 1**

| | Moisture content before drying (% by weight) | Drying condition | | | | | Dry-eliminated moisture content (% by weight) | Remaining moisture ratio (% by weight) | Amount of warpage (mm) | handleability |
|---|---|---|---|---|---|---|---|---|---|---|
| | | Location of microwave irradiation | Conveyor movement speed (m/min) | Microwave power (kW) | Hot air temperature (Degrees Celsius) | Hot air speed (m/sec) | | | | |
| Example 1 | 13.4 | upper and lower sides | 4.5 | 5 | 50 | 30 | 6.7 | 50 | 0.7 | ○ |
| Example 2 | 13.4 | upper and lower sides | 4.5 | 5 | 80 | 30 | 9.4 | 30 | 0.9 | ○ |
| Example 3 | 13.4 | upper and lower sides | 4.5 | 5 | 60 | 30 | 8.0 | 40 | 0.8 | ○ |
| Example 4 | 13.4 | upper and | 4.5 | 5 | 40 | 30 | 5.4 | 60 | 0.6 | Δ |
| Example 5 | 13.4 | upper and lower sides | 2.0 | 5 | 50 | 30 | 8.0 | 40 | 0.5 | ○ |
| Example 6 | 13.4 | upper and lower sides | 4.0 | 5 | 50 | 30 | 7.4 | 45 | 0.8 | ○ |
| Example 7 | 13.4 | upper and lower sides | 6.0 | 5 | 50 | 30 | 6.0 | 55 | 0.6 | ○ |
| Example 8 | 13.4 | upper and lower sides | 8.0 | 5 | 50 | 30 | 5.4 | 60. | 0.6 | Δ |
| Example 9 | 13.4 | upper and lower sides | 4.5 | 5 | 50 | 20 | 5.4 | 60 | 0.6 | Δ |
| Example 10 | 13.4 | upper and lower sides | 4.5 | 5 | 50 | 40 | 6.7 | 50 | 0.8 | ○ |
| Reference Example 1 | 13.4 | upper and lower sides | 4,5 | 5 | 100 | 30 | 10.7 | 20 | 1.1 | ○ |
| Reference Example 2 | 13.4 | upper and lower sides | 4.5 | 5 | 50 | 50 | 6.7 | 50 | 1.1 | ○ |
| Reference Example 3 | 13.4 | upper and lower sides | 4.5 | 5 | 30 | 30 | 4.0 | 70 | 0.5 | × |
| Reference Example 4 | 13.4 | upper and lower sides | 10.0 | 5 | 50 | 30 | 4.0 | 70 | 0.5 | × |
| Reference Example 5 | 13.4 | upper and lower sides | 4.5 | 5 | 50 | 10 | 4.0 | 70 | 0.5 | × |
| Comparative Example 1 | 13.4 | upper side upper side | 4.5 | 5 | 50 | 30 | 6.0 | 55 | 1.2 | ○ |

As is shown in Table 1, in the Examples, the handleability of the honeycomb molded body was satisfactory, having either no deformation or a deformation of less than 1 mm. And the amount of warpage of the honeycomb fired body was small, i.e., 0.8mm or less.
Alternately, in the Reference Examples 1 and 2, while the handleability of the honeycomb molded body was satisfactory, the amount of warpage of the honeycomb fired body was relatively great, i.e., at a value of 1.1mm. This is thought to have been caused by a sharp rise in the progression of the drying of the honeycomb molded body due to an excessively high heating temperature (Reference Example 1) and the airspeed of the hot air being too fast (Reference Example 2).

And in the Reference Examples 3 to 5, while the amount of warpage of the honeycomb fired body was as small as 0.5mm, handleability of the honeycomb molded body was inferior. This is thought to have been caused by insufficient progression of drying of the honeycomb molded body due to the temperature of the hot air being too low (Reference Example 3), the drying time being too short (Reference Example 4), and the air speed of the hot air being too slow (Reference Example 5).
And in the Comparative Example 1, although the handleability of the honeycomb molded body was satisfactory, the amount of warpage of the honeycomb fired body was great, i.e., at 1.2mm. This is thought to have been caused by the inability of drying to progress uniformly due to the microwaves being irradiated only from the upper side with respect to the honeycomb molded body.

### BRIEF DESCRIPTION OF THE DRAWINGS

Fig. 1 is a plan view showing a general representation of a drying apparatus of the present invention.
Fig. 2 (a) is a partial cross-sectional view taken along line A-A of the drying apparatus of the present invention shown in Fig. 1, and Fig. 2(b) is a partial cross-sectional view taken along line B-B of the drying apparatus of the present invention shown in Fig. 1.
Fig. 3 is a cross-sectional view schematically showing an example of a drying jig.
Fig. 4 is a perspective view schematically showing an example of a honeycomb structured body.
Fig. 5 (a) is a cross-sectional view schematically showing a honeycomb fired body constituting the honeycomb structured body, and Fig. 5 (b) is a cross-sectional view taken along line A-A of Fig. 5(a).
Fig. 6 (a) and 6(b) are schematic views describing an evaluation method of handleability.

### EXPLANATION OF SYMBOLS

- 10: Drying apparatus
- 11: Belt conveyor
- 13a to 13i: Microwave transmission portions
- 14a to 14i: Microwave irradiation parts
- 15a to 15d: Hot air blowing parts
- 15a' to 15d': Hot air aspiration parts
- 17: Microwave agitation blade
- 19: Drying furnace main body
- 20: Drying jig

## Claims

1. A drying apparatus comprising:
a plurality of microwave irradiation parts disposed alternately at the upper side and the lower side with respect to a conveying member for conveying an item to be dried; and
a plurality of hot air blowing parts,
wherein
the item to be dried is irradiated with microwaves in an alternating manner from the upper side and the lower side, and
hot air is applied in parallel with irradiation of the microwaves, to the item to be dried.

2. A drying method of a ceramic molded body comprising passing a ceramic molded body through the interior of a drying apparatus to dry said ceramic molded body, said passing carried out in a prescribed period of time by using a conveying member,
wherein
said drying apparatus comprises:
a plurality of microwave irradiation parts disposed alternately at the upper side and the lower side with respect to said conveying member; and
a plurality of hot air blowing parts, and
said drying apparatus irradiates said ceramic molded body with microwaves in an alternating manner from the upper side and the lower side, and carries out a hot air drying in parallel with irradiation of the microwaves.

3. The drying method of a ceramic molded body according to claim 2,
wherein
the moisture content of said ceramic molded body after drying is 30% by weight or more and less than 70% by weight of the moisture content before drying.

4. The drying method of a ceramic molded body according to claim 2 or 3,
wherein
the temperature of the hot air is in a range of 40 to 80 Degrees Celsius.

5. A method for manufacturing a honeycomb structured body comprising:
producing a pillar-shaped honeycomb molded body having a multiplicity of cells placed in parallel with one another in the longitudinal direction with a cell wall therebetween by molding a ceramic raw material;
carrying out drying of a molded body comprising passing said honeycomb molded body through the interior of a drying apparatus to dry said honeycomb molded body, said passing carried out in a prescribed period of time with the honeycomb molded body placed onto a conveying member; and
firing the dried honeycomb molded body to manufacture a honeycomb structured body comprising a honeycomb fired body,
wherein
said drying apparatus comprises:
a plurality of microwave irradiation parts disposed alternately at the upper side and the lower side with respect to said conveying member; and
a plurality of hot air blowing parts, and
said drying apparatus irradiates said honeycomb molded body with microwaves in an alternating manner from the upper side and the lower side, and carries out a hot air drying in parallel with irradiation of the microwaves.

6. The method for manufacturing a honeycomb structured body according to claim 5,
wherein
the moisture content of said honeycomb molded body after drying is 30% by weight or more and less than 70% by weight of the moisture content before drying.

7. The method for manufacturing a honeycomb structured body according to claim 5 or 6,
wherein
the temperature of the hot air is in a range of 40 to 80 Degrees Celsius.
